

## UNITED STATES PATENT OFFICE

FRANCIS JOHN SHEPHERD AND FRANK FORSTER RENWICK, OF LONDON, ENGLAND,  
ASSIGNORS TO ILFORD LIMITED, OF ILFORD, ENGLAND, A BRITISH COMPANY

## PHOTOGRAPHIC PRINTING PROCESS

No Drawing. Application filed August 29, 1930, Serial No. 478,800, and in Great Britain October 23, 1929.

This invention comprises improvements in or relating to photographic printing processes of the type known as the "Bromoil" process, according to which the following 5 method is adopted:—

A photographic print is made in the ordinary manner on a gelatin-silver-halide emulsion. In the process as hitherto carried out it is customary to employ a gelatin which is 10 soft and tender in character in the water-swelled condition. The print is developed in a non-tanning developer such as amidol, fixed, washed and immersed in a bleaching and tanning bath which has the property 15 of selectively hardening those portions of the gelatin which were in immediate contact with the metallic silver of the image, the rest of the gelatin remaining soft. The gelatin is then swelled by immersing the print in 20 warm water; and greasy ink is applied to the surface of the print by means of brushes, gradation being developed by carefully dotting on the ink, which is preferentially taken 25 up by the hardened portions of the gelatin and less readily or not at all by the softer and more swollen portions. The print so obtained may either constitute the final print itself, or may be used as a printer for transferring the ink to any desired surface, such 30 as a sheet of paper or the like.

The process described above suffers from the following disadvantages:—

1. Owing to the fact that the gelatin used in the emulsion must be very water absorbent in character, there is a large percentage of failures due to mechanical defects such as blistering, frilling and breakdown of the emulsion layer. 40  
2. In order to obtain an optimum swelling effect the swelling process which follows the tanning is usually carried out at a temperature well above normal i. e. exceeding 85° F. and the difficulty is that the best temperature is different for different types and ages of emulsion and must therefore be separately determined for each case. This procedure of varying the temperature of the bath by trial and error is extremely tedious and 45 unsatisfactory to carry out in practice.

3. The development of gradation by dotting ink on to the hardened portions of the gelatin layer by means of a brush takes a very considerable time. Owing to the ink repelling character and to the softness of 55 the swollen gelatin it is impossible in the usual Bromoil process to apply the ink satisfactorily by any more speedy method such for instance as by means of a roller.

4. The consistency of the ink employed in the Bromoil process may be varied somewhat to suit the degree of swelling of the gelatin but "hard" rapidly drying inks are unsuitable by themselves for the process, so that both 60 hard and soft (slow drying) inks are usually 65 employed either in admixture or in succession with the consequence that a long time, often several days, is required for the ink on the finished print to dry, whereas harder quicker drying inks are preferred for the 70 improved process described and much delay in the final drying process is thereby avoided.

5. It is necessary in the Bromoil process, but most difficult, particularly under certain 75 climatic conditions, to keep the print in a suitably damp condition throughout the prolonged inking process.

It is the object of the present invention to provide means whereby the above mentioned disadvantages of the Bromoil process hitherto used may be overcome.

The silver-halide-gelatin papers hitherto employed in the Bromoil process have been coated with an emulsion containing substantially no hardening agents, such as chrome 85 alum etc., in order to ensure that when the print is soaked in warm water immediately before the inking operation, there may be a marked differential swelling between the portions which have been tanned in the bleaching-hardening operation where the silver image previously existed, and the unhardened portions, which were free from image. If 90 the emulsion is too hard the whole area of the print takes up ink much too freely, and a satisfactory picture cannot be obtained. The melting point of the emulsion coating after swelling in water may be taken as a measure 95 of the hardness of the gelatin, and in the Bromoil process as carried out hitherto this 100

melting point has not usually exceeded 90-105° F.

According to the invention in a photographic printing process of the type described there is employed a silver-halide-gelatin emulsion comprising a prehardened gelatin, i. e., a gelatin whose melting point is above 105° F. Preferably the emulsion comprises a gelatin whose melting point exceeds 10 160° F.

According to a feature of the invention all the operations involving wetting of the print during its preparation from the unexposed silver-halide-gelatin emulsion up to the completion of the print are carried out at normal temperatures.

We have found that further difficulties arise in practice in printing processes of the "Bromoil" type particularly when the image 20 is bleached before fixing, owing to the fact that the bleaching baths employed are exceedingly sensitive in their attack on the silver image to variations in the hydrogen ion concentration of the surface of the print 25 upon which they act.

The developing solutions customarily employed in processes of the above type are alkaline in reaction, and very slight local variations in alkalinity such as may arise from 30 irregularities in the thickness of the gelatin layer, or from uneven washing after development, or even from the use of alkaline wash water when fixed bromide prints are washed and dried before bleaching are sufficient to 35 render it certain that the bleaching bath will not have a uniform action over the whole surface of the print, but will attack the silver image to different extents at different points on its surface. This in turn will give rise 40 to local irregularities in the ease with which the ink is taken up by the bleached print, and hence to unevennesses in the appearance of the finished print. It is a further object of 45 this invention to provide means whereby this difficulty may be overcome.

According to a further feature of the invention, applicable to that modification of a photographic printing process of the type described in which the bleaching operation 50 is carried out before the print is fixed, the print is brought, prior to bleaching, to a hydrogen ion concentration which is substantially uniform over its whole surface and comparable with (i. e. of substantially the 55 same order as) that of the bleaching bath to be employed.

According to yet another feature of the invention, the print after development, is transferred to a stop bath. By a stop bath 60 is to be understood a bath which has the effect of stopping the action of a preceding solution with which the print has been treated. Thus a stop bath for use after development normally comprises an acid solution 65 capable of neutralizing the alkaline devel-

oper, and thus preventing its further action on the print.

According to a feature of the invention, the stop bath may comprise a solution having a hydrogen ion concentration ranging from 10<sup>-4</sup> to 10<sup>-7</sup>, and a "buffering" action. By buffering action is to be understood the property of maintaining a substantially constant hydrogen ion concentration notwithstanding the addition of small quantities of acids or alkalies to the bath. Thus, for example, a solution of a salt of a weak acid, such for example as sodium acetate acts as a buffer as regards acids. If a little hydrochloric acid is added to this solution, the hydrogen ions liberated from the acid will combine with the CH<sub>3</sub>COO<sup>-</sup> ions liberated from the salts to form molecules of undissociated acetic acid, and the hydrogen ion concentration of the solution will remain substantially unaltered. By incorporating suitable mixtures of salts therein the solution may be buffered as regards both acids and alkalies.

In a preferred form of the invention the stop bath comprises an aqueous solution of borax and/or boric acid.

According to a further feature of the invention, ink is first uniformly applied to the bleached print, preferably after the latter has been dried, by means of a roller or an ink-spraying device or the like.

According to yet another feature of the invention gradation is developed in the print by damping the uniformly inked print, and rolling it with a wet roller of suitable material, e. g. india-rubber or felt, which picks up the ink from the non-tanned portions of the gelatin and transfers it preferentially to the tanned portions. The character of the gradation may be controlled locally by light 100 rolling of the damp print with an inky roller which thereby applies more ink to the tanned areas but not to the untanned areas and/or by slightly heavier rolling with a dry clean (uninked) roller of suitable material which 105 will remove any undesired excess of ink.

An example of the method of carrying the invention into practice will now be described.

A layer of silver-bromide-gelatin emulsion which has been pre-hardened in the course of manufacture by incorporating with it suitable hardening agents, e. g. chrome alum and/or formalin, is exposed to light under a negative, and developed by means of a non-tanning developer, such as metol quinol or amidol. In the case where amidol is employed the pH number of the developing solution is of the order of 7.5, whilst in the case of a metol quinol developer the pH number is as high as 9.6. The developed print is 110 then rinsed and transferred to the stop bath, which may be a cold saturated aqueous solution (i. e. an approximately 3% solution) of boric acid. This solution has a pH number 115 of about 5, and has the effect of bringing the 120

surface of the print to a uniform hydrogen ion concentration comparable with that of the bleaching bath, which may conveniently have a pH number of between 4 and 5. The 5 step of treating the print in the stop bath has the further advantage that it enables a bleaching bath of lower ion hydrogen concentration to be used than would otherwise be possible which greatly facilitates the subsequent inking operation.

After removal from the stop bath the print is transferred to a Bromoil bleaching and hardening bath of suitable hydrogen ion concentration (e. g. containing copper sulphate, 15 chromic acid and potassium bromide), washed well, fixed, washed again, and dried. The dry print is then uniformly inked by means of an ordinary gelatin or other elastic inking roller of the type used in photolithography. The ink may be any oily, fatty 20 or greasy ink, in which any suitable pigment may be incorporated; or if desired grease crayons may be employed for uniformly colouring the dry print. The print is then damped, either by a brief immersion in cold 25 water or by rolling with a wet fabric-covered roller. Gradation is then developed by rolling the print with a rubber or felt-covered roller, which causes the ink to be picked off the softer portions of the gelatin and transferred to the tanned portions. If desired further quantities of ink may be applied by 30 means of an ink covered roller or removed by a clean roller so that complete control over the depth of colouring of the print may be obtained. This adjustment of the gradation 35 may be carried out either under the surface of water in a suitable vessel, or on a glass slab or other smooth surface.

40 By means of the process according to the invention, it is an easy matter to ink a print measuring 12" x 10" in three to five minutes in full detail and depth of tone, whilst by means of the Bromoil process as hitherto employed, in which soaking in warm water 45 is necessary and inking is effected by means of brushes, it frequently takes from one to two hours to prepare a print of the same size.

The emulsion layers employed in carrying 50 into effect the process according to the invention may be carried on any suitable support such as paper, celluloid, glass, cellulose acetate, cellophane or the like.

The invention is also applicable to printing 55 processes of colour photography according to which two or more coloured images are combined together to give the finished picture either by super-position or by transfer to a common support.

60 The invention includes a photographic print when made by the special process described herein.

We claim:—

65 1. A process of the Bromoil type for obtaining a print in oil pigment on a non-re-

ticulated gelatin surface, which consists in forming the photographic print on a layer of silver-halide-gelatin emulsion which, by the addition of a hardening agent, has been pre-hardened to a degree such that its melting point is above 105° F., developing the print in a non-tanning developer, selectively hardening in a bleaching and tanning bath those portions of the gelatin which were in immediate contact with the metallic silver 70 of the image, applying greasy ink to the surface of the bleached fixed print, and developing gradation in the damp inked print by rolling it with a roller of material which will pick up ink from the non-tanned portions of the gelatin and transfer it preferentially to the tanned portions.

2. A process of the Bromoil type for obtaining a print in oil pigment on a non-reticulated gelatin emulsion surface, which consists in forming the photographic print on a layer of silver-halide-gelatin emulsion which by the addition of a hardening agent, has been pre-hardened to a degree such that its melting point is above 105° F., developing the print in a non-tanning developer, selectively hardening in a bleaching and tanning bath those portions of the gelatin which were in immediate contact with the metallic silver 80 of the image, applying greasy ink to the surface of the dry bleached fixed print, damping the inked print and developing gradation in the damp print by rolling it with a roller of material which will pick up ink from the non-tanned portions of the gelatin and transfer it preferentially to the tanned portions.

3. A process of the Bromoil type for obtaining a print in oil pigment on a non-reticulated gelatin surface, which consists in forming the photographic print on a layer of silver-halide-gelatin emulsion which, by the addition of a hardening agent, has been pre-hardened to a degree such that its melting point is above 105° F., developing the print in a non-tanning developer, selectively hardening in a bleaching and tanning bath those portions of the gelatin which were in immediate contact with the metallic silver 90 of the image, drying the print, applying greasy ink to the surface of the dry bleached fixed print, damping the inked print and developing gradation in the damp print by rolling it with a roller of material which will pick up ink from the non-tanned portions of the gelatin and transfer it preferentially to the tanned portions.

4. A process of the Bromoil type for obtaining a print in oil pigment on a non-reticulated gelatin surface, which consists in forming the photographic print on a layer of silver-halide-gelatin emulsion which, by the addition of a hardening agent, has been pre-hardened to a degree such that its melting point is above 105° F., developing the print in a non-tanning developer, selectively hardening in a bleaching and tanning bath those portions of the gelatin which were in immediate contact with the metallic silver 100 of the image, applying greasy ink to the surface of the bleached fixed print, and developing gradation in the damp inked print by rolling it in the cold with a roller of material which will pick up ink from the non-tanned portions of the gelatin and transfer it preferentially to the tanned portions.

105

110

115

120

125

130

ly hardening in a bleaching and tanning bath those portions of the gelatin which were in immediate contact with the metallic silver of the image, drying the print, applying 5 greasy ink to the surface of the dry bleached fixed print, damping the inked print and developing gradation in the damp print by rolling it in the cold with a roller of material which will pick up ink from the non-tanned portions of the gelatin and transfer 10 it preferentially to the tanned portions.

print and developing gradation in the damp inked print by rolling with a roller of material which will pick ink from the non-tanned portions of the gelatin and transfer it preferentially to the tanned portions.

70

5. A process of the Bromoil type for obtaining a print in oil pigment on a non-reticulated gelatin surface, which consists in forming the photographic print on a layer of silver-halide-gelatin emulsion which, by the addition of a hardening agent, has been pre-hardened to a degree such that its melting point is above 105° F., developing the print in a non-tanning developer, selectively hardening in a bleaching and tanning bath those portions of the gelatin which were in immediate contact with the metallic silver of the image, applying greasy ink to the surface of the bleached fixed print, and developing gradation in the inked print by rolling it under the surface of cold water in a suitable vessel with a roller of material which will pick up ink from the non-tanned portions of the gelatin and transfer it preferentially to the tanned portions.

8. A process of the Bromoil type for obtaining a print in oil pigment on a non-reticulated gelatin surface, which consists in forming the photographic print on a layer of silver-halide-gelatin emulsion which, by the addition of a hardening agent, has been pre-hardened to a degree such that its melting point is in the region of 160° F., developing the print in a non-tanning developer, selectively hardening in a bleaching and tanning bath those portions of the gelatin which were in immediate contact with the metallic silver of the image, applying greasy ink to the surface of the bleached, fixed print, and developing gradation in the damp inked print by rolling it in the cold with a roller of material which will pick up ink from the non-tanned portions of the gelatin and transfer it preferentially to the tanned portions.

75

35 entially to the tanned portions.

6. A process of the Bromoil type for obtaining a print in oil pigment on a non-reticulated gelatin surface, which consists in forming the photographic print on a layer of silver-halide-gelatin emulsion which, by the addition of a hardening agent, has been pre-hardened to a degree such that its melting point is in the region of 160° F., developing the print in a non-tanning developer, selectively hardening in a bleaching and tanning bath those portions of the gelatin which were in immediate contact with the metallic silver of the image, applying greasy ink to the surface of the bleached, fixed print and developing gradation in the damp inked print by rolling it with a roller of material which will pick up ink from the non-tanned portions of the gelatin and transfer it preferentially to the tanned portions.

9. A process of the Bromoil type for obtaining a print in oil pigment on a non-reticulated gelatin emulsion surface, which consists in forming the photographic print on a layer of silver-halide-gelatin emulsion which, by the addition of a hardening agent, has been pre-hardened to a degree such that its melting point is in the region of 160° F., developing the print in a non-tanning developer, selectively hardening in a bleaching and tanning bath those portions of the gelatin which were in immediate contact with the metallic silver of the image, drying the print, applying greasy ink to the surface of the dry bleached fixed print, damping the inked print and developing gradation in the damp print by rolling it in the cold with a roller of material which will pick up ink from the non-tanned portions of the gelatin and transfer it preferentially to the tanned portions. 90 95 100 105

88

55 7. A process of the Bromoil type for obtaining a print in oil pigment on a non-reticulated gelatin surface, which consists in forming the photographic print on a layer of silver-halide-gelatin emulsion, which by the addition of a hardening agent has been pre-hardened to a degree such that its melting point is in the region of 160° F., developing the print in a non-tanning developer, selectively hardening in a bleaching and tanning bath those portions of the gelatin which were in immediate contact with the metallic silver of the image, drying the print, applying greasy ink to the surface of the dry bleached fixed print, damping the inked

10. A process of the Bromoil type for obtaining a print in oil pigment on a non-reticulated gelatin surface, which consists in forming the photographic print on a layer of silver-halide-gelatin emulsion which, by the addition of a hardening agent, has been pre-hardened to a degree such that its melting point is in the region of 160° F., developing the print in a non-tanning developer, selectively hardening in a bleaching and tanning bath those portions of the gelatin which were in immediate contact with the metallic silver of the image, applying greasy ink to the surface of the bleached fixed print, and developing gradation in the inked print by rolling it under the surface of cold water in a suitable vessel with a roller of material which will pick up ink from the non-tanned portions of the gelatin and transfer it preferentially to the tanned portions. . . .

115

## 11. A process of the Bromoil type for ob- 130

taining a print in oil pigment on a non-reticulated gelatin surface, which consists in forming the photographic print on a layer of silver-halide-gelatin emulsion which, by the 5 addition of a hardening agent has been prehardened to a degree such that its melting point is above 105° F., developing the print in a non-tanning developer, transferring the print to a stop bath having a hydrogen ion 10 concentration ranging from  $10^{-4}$  to  $10^{-7}$  and a buffering action, selectively hardening in a bleaching and tanning bath those portions of the gelatin which were in immediate contact with the metallic silver of the image, fixing 15 the print, applying greasy ink to the surface of the bleached fixed print and developing gradation in the damp inked print, by rolling it with a roller of material which will pick up ink from the non-tanned portions of the gelatin and transfer it preferentially to the 20 tanned portions.

12. A process of the Bromoil type for obtaining a print in oil pigment on a non-reticulated gelatin surface, which consists in 25 forming the photographic print on a layer of silver-halide-gelatin emulsion, which by the addition of a hardening agent has been prehardened to a degree such that its melting point is above 105° F., developing the print in 30 a non-tanning developer, fixing the print, transferring the print to a stop bath having a hydrogen ion concentration ranging from  $10^{-4}$  to  $10^{-7}$  and a buffering action, selectively hardening in a bleaching and tanning bath 35 those portions of the gelatin in immediate contact with the metallic silver of the image, applying greasy ink to the surface of the bleached fixed print, and developing gradation in the damp inked print by rolling it 40 with a roller of material which will pick up ink from the non-tanned portions of the gelatin and transfer it preferentially to the tanned portions.

45 13. A process of the Bromoil type for obtaining a print in oil pigment on a non-reticulated gelatin surface, which consists in forming the photographic print on a layer of silver-halide-gelatin emulsion which, by the 50 addition of a hardening agent, has been prehardened to a degree such that its melting point is above 105° F., developing the print in a non-tanning developer, fixing the print, transferring the print to a stop bath having 55 a hydrogen ion concentration varying from  $10^{-4}$  to  $10^{-7}$  and a buffering action, selectively hardening in a bleaching and tanning bath those portions of the gelatin which were in immediate contact with the metallic silver of 60 the image, drying the print, applying greasy ink to the surface of the print by means of a roller, damping the print, and developing gradation in the damp inked print by rolling it with a roller of material which will pick up 65 ink from the non-tanned portions of the gel-

tin and transfer it preferentially to the tanned portions.

14. A process of the Bromoil type for obtaining a print in oil pigment on a non-reticulated gelatin surface, which consists in forming 70 the photographic print on a layer of silver-halide-gelatin emulsion which, by the addition of a hardening agent, has been prehardened to a degree such that its melting point is above 105° F., developing the print in a non-tanning developer, transferring the print to a stop bath having a hydrogen ion concentration varying from  $10^{-4}$  to  $10^{-7}$  and a buffering action, selectively hardening in a bleaching and tanning bath those portions of the gelatin 75 which were in immediate contact with the metallic silver of the image, fixing the print, drying the print, applying greasy ink to the surface of the print by means of a roller, damping the print, and developing gradation 80 in the damp inked print by rolling it with a roller of material which will pick up ink from the non-tanned portions of the gelatin and transfer it preferentially to the tanned 85 portions.

In testimony whereof we have signed our names to this specification.

FRANCIS JOHN SHEPHERD.  
FRANK FORSTER RENWICK.

90

95

100

105

110

115

120

125

130